

June 30, 1931.

W. EHLERS

1,812,740

MAGNET CORE

Filed June 26, 1926



Inventor:  
Walther Ehlers  
by *Steinboeck*  
Atty.

## UNITED STATES PATENT OFFICE

WALTHER EHLERS, OF BERLIN-COPENICK, GERMANY, ASSIGNOR, BY MESNE ASSIGNMENTS, TO GENERAL ELECTRIC COMPANY, A CORPORATION OF NEW YORK

## MAGNET CORE

Application filed June 26, 1926, Serial No. 118,742, and in Germany July 6, 1925.

My invention refers to magnet cores, more especially such as form part of induction coils of the Pupin system. It is an object of my invention to provide a magnet core which is adapted to fulfill the varying requirements regarding its magnetic and electric properties, which are made according to the particular purpose for which the coil is used.

10 Hitherto each magnet core was made of some uniform material, either in one piece or in several pieces of equal shape, and in order to satisfy the varying requirements mentioned above either the quality of the 15 cores was modified or else some standard types were used for every purpose without taking regard to the most favorable quality in each case.

Obviously the difficulty in providing in 20 each individual case a core which fulfills all requirements becomes greater every day and renders it almost impossible to keep such cores in store.

According to the present invention now, I 25 build up the core from several units, but in contradistinction to this well known step the core according to my invention is built up from units possessing different electric and magnetic properties, such as are required in each individual case to render the 30 core adapted to fulfill all requirements of the case. I thus render it possible to keep in store certain units having predetermined electric and magnetic properties, and I am 35 therefore enabled to compose any special core that may be ordered, by merely selecting the corresponding units.

As is well known to those skilled in the 40 art the requirements made regarding the magnetic and electric properties of the cores of Pupin coils are substantially the following:

- 45 (a) Permeability,
- (b) Stability,
- (c) Lowest eddy current losses,
- (d) Lowest hysteresis losses.

Assuming for instance a core to be prepared having the largest possible permea-

bility ( $\mu$ ), and a stability in which  $\frac{\Delta\mu}{\mu}$  (variation of  $\mu$  under direct current load up to 0,1 ampere) is less than 1 per cent, the losses by eddy currents  $W$  being smaller than  $9 \Omega/\text{Henry}$ , and the losses by hysteresis  $h$  less than  $50 \text{ ohm}/\text{Henry}/\text{amp}/\text{cms}$ .

Assuming further the following groups of units to be available for fulfilling these requirements, viz.: 60

(1) Hard steel wire

$$\mu = 100, \frac{\Delta\mu}{\mu} = -1\%, W = 20, h = 150,$$

(2) Solid core

$$\mu = 35, \frac{\Delta\mu}{\mu} = +1\%, W = 5, h = 10.$$

If now, according to the drawing annexed 70 to this specification and forming part thereof, which is a diagrammatic view of a core by way of example, the core is composed of four annular discs of uniform size, one of which (the uppermost) disc (a) is made 75 of the material of group 1 (hard steel wire), while the three other (b) belong to group 2, the composite core will have the following properties:

$$\mu = \frac{1}{4} (1 \cdot 100 + 3 \cdot 35) = 51$$

$$\text{Stab.} = 100 \frac{\frac{1}{4} (1 - 1 + 3 \cdot 0,35)}{\frac{1}{4} (1.100 + 3 \cdot 35)} = +0,025\%$$

$$W = \frac{1}{4} (1 \cdot 20 + 3 \cdot 5) + 8,8$$

$$h = \frac{1}{4} (1 \cdot 150 + 3 \cdot 10) = 45.$$

The effective permeability  $\mu = 51$ , which is obtained according to the above, cannot practically be obtained by any means hitherto known, if the limits of stability and losses are taken into consideration.

I wish it to be understood that I do not desire to be limited to the exact details of construction shown and described for obvious modifications will occur to a person skilled in the art.

I claim:—

1. Magnet core composed of a plurality of superposed units offering an uninterrupt-

80

65

70

75

80

85

90

95

100

ed path to the magnetic flux and consisting of magnetic material having a marked permeability, one of said units differing from another unit in its magnetic properties.

5 2. Magnet core composed of a plurality of superposed units offering an uninterrupted path to the magnetic flux and consisting of magnetic material having a marked permeability, one of said units differing from another unit in its magnetic and electrical properties.

10 3. Magnet core composed of a plurality of superposed annular units offering an uninterrupted path to the magnetic flux and consisting of magnetic material having a marked permeability, one of said units differing from another unit in its magnetic properties.

15 4. Magnet core composed of a plurality of superposed annular units offering an uninterrupted path to the magnetic flux and consisting of magnetic material having a marked permeability, one of said units differing from another unit in its magnetic and electrical properties.

20 25 In testimony whereof I affix my signature.

WALTHER EHLERS.

30

35

40

45

50

55

60

65